

July 4, 1944.

H. B. RICHMOND ET AL

2,352,658

METHOD OF COATING PAPER

Filed Sept. 26, 1941

FIG. 2.



FIG. 1.



Inventors:  
Howard Brewster Richmond,  
Gilbert K. Dickerman.  
By: Lee J. Gary  
Attorney.

## UNITED STATES PATENT OFFICE

2,352,658

## METHOD OF COATING PAPER

Howard Brewster Richmond and Gilbert K. Dickerman, Wisconsin Rapids, Wis., assignors to Consolidated Water Power & Paper Company, Wisconsin Rapids, Wis., a corporation of Wisconsin

Application September 26, 1941, Serial No. 412,362

12 Claims. (Cl. 117—111)

This invention relates to improvements in a method of coating paper, paperboard or the like, with a mineral coating material by means of rolls to provide a coated surface upon the web which is ideally adapted for printing purposes, and refers specifically to the control of the relative peripheral speeds of the coating roll or rolls and the translatory speed of the web to be coated and the relative peripheral speed of the rolls with respect to each other in order that a smooth uniform film may be applied to the web surface.

The manufacturers of mineral coated papers and paperboard by roll processes have long encountered two serious production problems:

1. The occurrence on the coated surface of blemishes or irregularities resembling the pattern of a cat's paw. These blemishes are sometimes referred to in the art as "cat tracks."

2. The difficulty in preparing a coated paper or paperboard in which both sides of the web have the same surface characteristics. The wire side of the web is usually rougher than the felt side and, hence, if both sides are coated with the same amount of coating material, the opposite faces of the web will have different characteristics. This problem is known in the art as "two-sidedness." The seriousness of this problem in the production of two-sided coated webs for books, magazines, cartons, and the like, is apparent.

We have found that the nucleus of the "cat track" is a small particle of solid coating material lodged on the surface of one or both of the coating applying rolls. As the surface of the web is brought into contact with a coating roll containing such solid particle the coating is formed imperfectly around this nucleus. As the web leaves the coating roll a definite pattern is made at the point of this nucleus in the coated surface.

We have found that "cat tracks" can be eliminated by the correlation of the peripheral speeds of the coating rolls with respect to the translatory speed of the web. That is, by driving the coating rolls at a peripheral speed greater or less than the translatory speed of the web, the wiping action thus brought about obliterates the "cat tracks."

The most expeditious way of curing the defect of "two-sidedness" is to apply more coating material to the wire side of the web than to the felt side thereof. Because of difficulties brought about by applying unequal amounts of coating material to the opposite sides of the web, expensive auxiliary coating apparatus has heretofore

been deemed necessary in order to solve the problem. We have found, however, that a proper correlation of the peripheral speed of the rolls and the translatory speed of the web solves the problem of "two-sidedness" without the use of supplementary equipment.

Another important factor in the production of a properly coated web is the "draw," that is, the tension of the web in passing through the coating unit. If the coating roll or rolls are run at the same peripheral speed as the speed of the web, the draw will not be affected. However, if the rolls are run at peripheral speeds different from the speed of the web, and the speeds are not properly correlated, the draw will be disturbed and the web will break or wrinkle, negating a smoothly coated web.

Therefore, it is obvious that in eliminating "cat tracks" and curing two-sidedness by varying the speed of the rolls with respect to the speed of the web, a new problem, the draw, arises.

Hence, our invention is not only directed to the correlation of the speed of the rolls with respect to the web, but also the correlation of the speed of the rolls with respect to each other.

The objects and advantages of our invention will be apparent from the accompanying drawing and following detailed description.

In the drawing,

30 Fig. 1 is a diagrammatic view of two juxtaposed coating rolls driven at equal peripheral speeds and substantially equal to the translatory speed of the web.

35 Fig. 2 is a similar view with the lower roll driven at a peripheral speed higher than that of the upper roll and greater than the translatory speed of the web.

40 Referring in detail to the drawing, 1 indicates the upper roll and 2 indicates the lower roll of a pair of juxtaposed rolls between which a web 3 passes. The rolls 1 and 2 may have applied to either, or both of their surfaces, by means of one or more contacting rolls (not shown) or otherwise, a mineral coating material. This type of coating unit is well known to the art, the web 3 passing between the rolls 1 and 2 being coated on one or both surfaces.

45 For purposes of description both rolls 1 and 2 will be considered as coating rolls and the web 3, which may be paper or paperboard, will be coated simultaneously on both surfaces. Of course, our invention contemplates the coating of either one side or the other of the web as a separate operation or the coating of both sides simultaneously, as herein described.

When roll 1 travels at the same peripheral speed as the translatory speed of the web and at the same peripheral speed as roll 2, the web 3 after leaving the nip usually tends to adhere to the surface of roll 1, as indicated at 4. When the web finally leaves the surface of roll 1 it does so in a more or less abrupt manner, leaving on the web an irregular pattern or "cat track." This pattern or "cat track" results from imperfect formation of the coating on the web caused by a particle of solid material lodged on the surface of the coating rolls resulting in imperfect formation of coating on the rolls at this point.

This condition can be cured by rotating the roll 1 at a peripheral speed greater or lesser than the translatory speed of the web. In so doing a wiping action is brought about which smooths the coated surface and thus removes the "cat track" formed. We have found the web normally adheres to the surface which is moving at a greater peripheral speed. Hence, although the web may normally adhere to the upper roll surface, it can be made to adhere to the lower roll surface by causing the lower roll to move at a peripheral speed greater than that of the upper roll. However, regardless of whether the web adheres to one roll or the other after leaving the nip, the differential in surface speed between said rolls and the web obliterates "cat tracks."

Under normal conditions the web consistently adheres, in passing between coating rolls to one or the other of the rolls for a longer distance beyond the nip. This is believed to be due to capillary attraction which may result from the roll to which the web adheres being smoother than the other roll, or one surface of the web being smoother than the other, the smoother web surface tending to adhere to the adjacent coating roll longer than the rougher surface adheres to its adjacent roll. In most instances it has been found that the web has a greater tendency to adhere to the upper roll, and in the subsequent discussion of our invention this condition will be considered as obtaining.

Normally, the lower surface of the web 3 is rougher than the upper surface, and contains wire marks from the forming wire. It is desirable to obscure these marks by applying a greater weight of coating to the wire side of the web. Prior to our invention roll coater operators found it necessary to apply an equal amount of coating to each coating roll in order to assure the web would have a consistent travel through the coating unit. It was found that the mere application of a greater amount of coating to the bottom roll than to the top roll would cause the web, after passing through the nip of the coating rolls or through the nip of the coating roll and back-up roll (if a single side coater is operated), to "flop" back and forth from top to bottom roll, adhering neither to the bottom nor to the top roll consistently, thus causing streaks or mars on the coated surface. Our invention in this respect consists of driving the lower roll (2) at a greater peripheral speed than the speed of the upper roll and in addition applying a greater quantity of coating to the bottom roll. These two factors cause the web to consistently adhere to the bottom roll for a few inches after passing through the nip (shown best at 5 in Fig. 2) thus accomplishing our purpose of correcting two-sidedness without additional coating equipment and still maintaining a stable production condition.

It can readily be seen that by establishing a differential in surface speed between, for in-

stance, the web and the lower coating roll, more coating material can be applied to the lower surface of the web while maintaining the web adhering consistently to the lower roll. Two-sidedness can therefore be cured and simultaneously "cat tracks" which may tend to form are eliminated.

However, a third factor must be considered and that is the draw. Generally speaking the draw is the condition of tension in the web which moves it forwardly between two points in the paper machine. In passing the web between the coating rolls 1 and 2, the surface speed of said rolls being the same as the speed of the web, the draw will not be disturbed. However, if one of said rolls is driven at a speed different from the speed of the web and the other roll maintained at web speed, the draw will be disturbed and the web will tend to wrinkle or break.

Hence, in the situation where the speed of the lower roll is different from the speed of the web to cure two-sidedness and eliminate "cat tracks," and the surface speed of the upper roll is maintained at the speed of the web, the draw is disturbed.

As another feature of our invention, we contemplate varying the surface speed of each roll with respect to the speed of the web and also with respect to each other. We have found that when the surface speed of one roll, for instance roll 2, is increased say 5 percent, with respect to the speed of the web, a proper and satisfactory draw can be maintained by decreasing the surface speed of the roll 1 about 5 percent with respect to the speed of the web. This change in surface speed of the upper roll with respect to the web not only compensates for any disturbance to the draw caused by the lower roll, but roll 1, moving at a surface speed slower than the speed of the web tends to obliterate "cat tracks" which may otherwise be formed on the upper surface of the web.

We have found that either roll may be driven at a surface speed between .25 and 10 per cent different from the translatory speed of the web. Preferably, however, a speed differential of between .5 and 1.5 is deemed most satisfactory. By maintaining a speed differential within the range specified, "cat tracks" and "two-sidedness" can be cured without rendering the operation too critical.

For example, the speed of the web 3 may be 815 feet per minute; the peripheral speed of roll 1 may be 800 feet per minute and the peripheral speed of roll 2 may be 830 feet. In other words, roll 1 may run 1.88 per cent slower than web 3 and roll 2 may run 1.88 per cent faster than web 3, and roll 2 may run 3.76 per cent faster than roll 1.

A third factor enters into the problem, however, which must be observed and this factor limits the relationship of the various speeds involved. This factor is the "draw." It is preferable that for an ideal draw, the speed of the web be maintained about midway between the peripheral speeds of the rolls, that is, that the speed differential percentage of one roll with respect to the web be substantially equal to the speed differential percentage of the other roll with respect to the speed of the web, said speed differentials being of opposite sign. However, the surface speed differential or percentage of difference in speed of one roll with respect to the speed of the web should not exceed by at most about 5 per cent and preferably not over 1.8 per cent the surface speed differential of the

other roll with respect to the web, the speed differentials being of opposite sign.

Within the limits stated herein, the following factors are of importance: The furnish of the web or sheet; the weight of the sheet; the absorptiveness of the sheet; the smoothness of the surface of the sheet; the amount of coating applied, and the viscosity and solids content of the coating material.

In general, the hereinbefore-mentioned factors influence the relative speed of the rolls and web and the relative speed of the rolls with respect to each other, as follows: With regard to the furnish of the sheet, a sulphite sheet is generally less absorptive than a groundwood sheet and normally the greater the percentage of groundwood in a sheet the greater is its absorptiveness. The more absorptive the sheet the faster the coating material is dehydrated when applied. The side of the sheet on which the coating is most dehydrated, other factors being equal, will adhere to the coating roll after leaving the nip. Generally, therefore, to cause the absorptive sheet to adhere to a predetermined roll when it normally tends to adhere to the other roll, requires a greater speed differential than would be the case with a less absorptive sheet. In addition, a sheet having a partially dehydrated coating has a more sticky surface characteristic than a less dehydrated coated surface, and, hence, a greater speed differential between roll and sheet is required to remove cat tracks.

Of course, in view of the fact that speed differentials of the rolls with respect to the web and with respect to each other result in friction at the nip, greater speed differentials may be employed with stronger or heavier sheets, and lighter weight or weaker sheets dictate the use of lesser speed differentials.

The absorptiveness of the sheet has hereinbefore been discussed with respect to the furnish of the sheet, and with respect to the smoothness of the sheet, generally stated, the smoothest side of the sheet tends to adhere to the roll. Normally, the smoothest side of the sheet is the most absorptive side thereof.

In view of the fact that the coating material tends to function as a lubricant at the nip and promote slippage, the greater the weight of coating, the greater speed differentials may be resorted to which is highly desirable; and vice versa, the lighter the weight of coating the lesser the speed differentials are which can be employed successfully with a sheet of predetermined weight.

Generally, the more fluid the coating, the less speed differential is required to obliterate cat tracks and obtain a proper draw. The greater the viscosity and solids content of the coating, the greater are the speed differentials necessary to accomplish the same results.

All of these factors must be taken into consideration in determining the optimum operating conditions within the range hereinbefore set forth. Below the lower limits set forth, no appreciable results are attainable in eliminating "cat tracks" and obliterating wire marks, and above the upper limits specified all of the factors hereinbefore set forth, as well as others, become so critical that commercial operation is substantially impossible.

We claim as our invention:

1. In a method of coating paper, paper board and the like felted fibrous webs wherein the web

75

is passed between juxtaposed rolls rotating in opposite directions at least one of which carries a mobile coating material upon its surface which is deposited upon a surface of the web, the improvement which comprises, driving each of the rolls at a surface speed of opposite sign of about .25 per cent to 10 per cent different from the translatory speed of the web.

2. In a method of coating paper, paper board and the like felted fibrous webs wherein the web is passed between juxtaposed rolls rotating in opposite directions at least one of which carries a mobile coating material upon its surface which is deposited upon a surface of the web, the improvement which comprises, driving the coating roll at a surface speed of about .25 per cent to 10 per cent faster and the other roll approximately the same percentage slower than the translatory speed of the web.

15 3. In a method of coating paper, paper board and the like felted fibrous webs wherein the web is passed between juxtaposed rolls rotating in opposite directions at least one of which carries a mobile coating material upon its surface which is deposited upon a surface of the web, the improvement which comprises, driving the coating roll at a surface speed of about .25 per cent to 10 per cent slower and the other roll approximately the same percentage faster than the translatory speed of the web.

20 4. In a method of coating paper, paper board and the like felted fibrous webs wherein the web is continuously passed between juxtaposed coating rolls rotating in opposite directions and a mobile coating material is continuously deposited upon the surface of said coating rolls and transferred to opposed surfaces of said passing web, the improvement which comprises, driving each of said rolls at a surface speed of opposite sign of about .25 per cent to 10 per cent different from the translatory speed of the web.

25 5. In a method of coating paper, paper board and the like felted fibrous webs wherein the web is continuously passed between juxtaposed coating rolls rotating in opposite directions and a mobile coating material is continuously deposited upon the surface of said coating rolls and transferred to opposed surfaces of said passing web, the improvement which comprises, driving each of said rolls at a surface speed of opposite sign of about .25 per cent to 10 per cent different from the translatory speed of the web to thereby substantially equalize tension on the web.

30 6. In a method of coating paper, paper board and the like felted fibrous webs wherein the web is continuously passed between juxtaposed coating rolls rotating in opposite directions and a mobile coating material is continuously deposited upon the surface of said coating rolls and transferred to opposed surfaces of said passing web, the improvement which comprises, driving one of said rolls at a surface speed of about .25 per cent to 10 per cent different from the translatory speed of the web, and driving the other roll at a surface speed different from the translatory speed of the web, the percentage of difference in speed of each of said rolls with respect to said web speed being substantially equal and of opposite sign.

35 7. In a method of coating paper, paper board and the like felted fibrous webs wherein the web is continuously passed between juxtaposed rolls rotating in opposite directions and a mobile coating material is continuously deposited upon the surface of one of said rolls and transferred to a surface of said passing web, the improvement which comprises, driving one of said rolls at a surface speed of about .25 per cent to 10 per cent different from the translatory speed of the web, and driving the other roll at a surface speed similarly different from the translatory speed of the web, the percentage of difference in speed of one of said rolls with respect to the web speed being not in excess of about 5 per cent of that of the other and of opposite sign.

40 8. In a method of coating paper, paper board

and the like felted fibrous webs wherein the web is continuously passed between a pair of superimposed coating rolls rotating in opposite directions and a mobile coating material is continuously deposited upon the surface of said coating rolls and transferred to opposed surfaces of said passing web, the improvement which comprises, driving the lower roll at a surface sped of about .25 per cent to 10 per cent faster than the surface speed of the web and about twice said per cent faster than the surface speed of the upper roll to eliminate "cat tracks" on the coated surface and obliterate wire marks on the web.

8. In a method of coating paper, paper board and the like felted fibrous webs wherein the web is passed between juxtaposed rolls rotating in opposite directions at least one of which carries a mobile coating material upon its surface which is deposited upon a surface of the web, the improvement which comprises, driving each of the rolls at a surface speed of opposite sign of about .5 per cent to 1.5 per cent different from the translatory speed of the web.

9. In a method of coating paper, paper board and the like felted fibrous webs wherein the web is continuously passed between juxtaposed coating rolls rotating in opposite directions and a mobile coating material is continuously deposited upon the surface of said coating rolls and transferred to opposed surfaces of said passing web, the improvement which comprises, driving one of said rolls at a surface speed of about .5 per cent to 1.5 per cent different from the translatory speed of the web, and driving the other roll at a surface speed of about .5 per cent to 1.5 per cent different from the translatory speed of the web, the relative speed percentages of said rolls being of opposite sign.

10. In a method of coating paper, paper board and the like felted fibrous webs wherein the web is continuously passed between superimposed coating rolls rotating in opposite directions and a mobile coating material is continuously deposited upon the surface of said coating rolls and transferred to opposed surfaces of said passing web, the improvement which comprises, driving the lower roll at a surface speed of about .5 per

cent to 1.5 per cent faster than the translatory speed of the web, and about twice said per cent faster than the surface speed of the upper roll to eliminate "cat tracks" on the coated surface and obliterate wire marks on the lower surface of the web.

11. In a method of coating paper, paper board and the like felted fibrous webs wherein the web is continuously passed between a pair of juxtaposed rolls rotating in opposite directions and a mobile coating material is continuously deposited upon the surface of one of said coating rolls and transferred to a surface of said web, the improvement which comprises, driving one of said rolls at a surface speed of about .25 per cent to 10 per cent different from the translatory speed of the web, and driving the other roll at a surface speed different from the translatory speed of the web, the speed difference percentage of one of said rolls with respect to said web being not greater than about 5 per cent different from the speed difference percentage of the other roll with respect to said web, the speed percentage differences between said rolls and said web being of opposite sign.

12. In a method of coating paper, paper board and the like felted fibrous webs wherein the web is continuously passed between a pair of juxtaposed rolls rotating in opposite directions and a mobile coating material is continuously deposited upon the surface of one of said coating rolls and transferred to a surface of said web, the improvement which comprises, driving one of said rolls at a surface speed of about .25 per cent to 10 per cent different from the translatory speed of the web, and driving the other roll at a surface speed different from the translatory speed of the web, the speed difference percentage of one of said rolls with respect to said web being not greater than about 1.8 per cent different from the speed difference percentage of the other roll with respect to said web, the speed percentage differences between said rolls and said web being of opposite sign.

45 HOWARD BREWSTER RICHMOND.  
GILBERT K. DICKERMAN.